

## 1

3,687,720

### PROCESS FOR FLAMEPROOFING TEXTILE MATERIAL

Werner Grunewalder, 89 Am Falder,  
4 Dusseldorf-Holthausen, Germany

No Drawing. Filed Nov. 26, 1969, Ser. No. 880,377  
Claims priority, application Germany, Dec. 6, 1968,  
P 18 13 021.7

Int. Cl. C09d 5/18

U.S. CL. 117—137

2 Claims 10

#### ABSTRACT OF THE DISCLOSURE

Describes a process for flameproofing textiles in which substantially anhydrous zinc chloride in substantially anhydrous solvents is used as the flameproofing material, the substantially anhydrous flameproofing composition prevents creasing and shrinking of the treated textiles.

The invention relates to a process for flameproofing textiles.

It is known to treat textile materials made of readily inflammable cellulose fibres with a flameproofing treatment with aqueous solutions or emulsions of various inorganic or organic compounds. In particular, already made up textiles, such as for example, curtains, protective clothing, special military textiles and the like are given such treatment. It has been found, however, that the known processes working with aqueous solutions or emulsions are not only complicated and time consuming, but also lead to damage of the cellulose textiles, since owing to the wet treatment, these tend to crease and shrink to a considerable extent.

An object of the present invention is to provide a flameproofing process for cellulose textiles which will not materially crease or shrink the fabric.

Another object of the invention is to provide a process for flameproofing cellulose textiles which can be used in the cleaning machines ordinarily used in chemical cleaning, and may be preceded with or followed with chemical cleaning or the cleaning may take place simultaneously, in the same machine.

Another object is to provide a substantially anhydrous flameproofing concentrate which when mixed with substantially anhydrous solvents used in the preparation of the flameproofing baths will give a substantially clear solution which will not tend to crease and shrink already made up cellulose textiles.

Various other objects and advantages of the invention will appear as this description proceeds.

The present invention, therefore, provides an impregnating bath medium, for flameproofing cellulose textiles, comprising a mixture of a substantially anhydrous zinc chloride in a lower alcohol, glycol or carboxylic acid ester and an organic solvent utilizable for chemical cleaning. The bath medium should be substantially anhydrous, having a low water content in the entire bath composition.

The process for flameproofing textiles which consist wholly or substantially of cellulose or regenerated cellulose fibres provided herein, comprises contacting said textiles with a bath medium comprising a mixture of a concentrated substantially anhydrous solution of zinc chloride in a lower alcohol, glycol or carboxylic acid ester and a substantially anhydrous organic solvent utilizable for chemical cleaning.

In order to prepare the impregnating baths, a concentrated stock solution is first made by dissolving zinc chloride in an anhydrous lower alcohol or glycol containing 2 to 4 carbon atoms, such as ethanol, propanol, isopropanol, butanol, ethylene glycol, 1,3- or 1,3-propylene

## 2

glycols and the like. Further suitable solvents are esters of the said alcohols with monocarboxylic acids which contain 1 to 4 carbon atoms, as for example, ethyl acetate, the monoglycol ester of propionic acid and the like. These concentrates contain 5 to 35% by weight of anhydrous zinc chloride, which may consist either of products of technical purity with the lowest possible content of coloring or sludge-forming impurities, or if desired products of high purity, for example, corresponding to the German pharmacopoeia quality "DAB 6".

10 to 60 g. per liter, calculated on anhydrous zinc chloride, of the said concentrates are added to the organic solvents to form an impregnating bath. The impregnating liquors consist of the solvents utilized in chemical cleaning, especially petroleum hydrocarbons of boiling points of 80° to 200° and halogenated hydrocarbons having 1 to 4 carbon atoms such as methylene chloride, carbon tetrachloride, perchlorethylene, trifluorotrichloroethane, monofluorotrichloromethane, etc.

20 These solvents should be largely water-free. It has surprisingly been found that the said concentrates containing zinc chloride can be mixed with the solvents used for the preparation of impregnating baths giving clear or slightly turbid solutions. These baths are also sufficiently stable.

25 The process is effected preferably in the cleaning machines used in chemical cleaning, suitably following a chemical cleaning. The textiles are treated with the impregnant medium at 20° to 35° C. for 2 to 10 minutes and after centrifuging and drying are ready for use. 30 Depending on the amount of zinc chloride applied to the textile fibres, very good flameproofing effects can be attained which correspond to the DIN specifications 53,906 and 53,907. In general, an application of 0.8 to 8% by weight of zinc chloride, based on the weight of the fibre, is needed.

35 In order to assist the effect, further known organic flameproofing agents, provided they are soluble in the impregnating liquors, may be added to the baths. For example, halogenated paraffins, especially chlorinated paraffins, which simultaneously exert a specific softening action on the textile fibre, are suitable for this purpose. These ingredients are added to the baths in amounts of from 3 to 20 g. per liter. Apart from these, further additions customary in textile finishing may also be present, such as brightening agents, waterproofing agents, dressing agents or agents producing a high finish, for example, urea or melamine-formaldehyde condensation products and the like.

#### EXAMPLE 1

50 In a cleaning machine of the "Böwe R 9 M" type, 6 kg. of curtains, consisting of rayon staple fibre rep, were cleaned as usual and then treated for 5 minutes in 60 liters of perchlorethylene with the addition of 10 liters 55 of butyl acetate in which 12% by weight of anhydrous zinc chloride was dissolved. The textiles so treated, after centrifuging and drying in the cleaning machine, were difficultly inflammable, in contrast to untreated curtains.

#### EXAMPLE 2

60 In the cleaning machine used in Example 1, 8 kg. of working clothes, consisting of cotton twilled fabric, were chemically cleaned and then flameproofed. The flameproofing was carried out by treating the fabric for 5 minutes in 60 liters of trichloroethylene with an addition of 12 liters of ethyl glycol, in which 15% of anhydrous zinc chloride was dissolved. After centrifuging until the residual moisture was 80%, the suits were dried with hot air. The estimation of the flameproofing effect was carried out, after air conditioning under standard conditions according to the DIN specification 53,907. In compari-

son with untreated goods, the following values were obtained:

TABLE I

| Cotton twill   | Diameter of hole, mm. |                       |                  |          |
|----------------|-----------------------|-----------------------|------------------|----------|
|                | Burning time, seconds | Glowing time, seconds | Small-est        | Larg-est |
| Treated.....   | 3                     | 5                     | 10               | 30       |
| Untreated..... | (1)                   | (1)                   | Completely burnt |          |

<sup>1</sup> Deflagrated.

It can be seen from the values in the table that the treated cotton twill fabric is difficultly inflammable.

## EXAMPLE 3

2 kg. of staple fibre gabardine were treated for 5 minutes in 20 liters of monofluorotrichloromethane with the addition of 3 liters of isopropanol, in which 15% of anhydrous zinc chloride (DAB 6) and 10% of coconut fatty acid polydiethanolamide were dissolved. The material was then centrifuged and dried as usual. The treated material in contrast to the untreated goods, was only difficultly inflammable and had a soft handle.

## EXAMPLE 4

25 kg. of welders' protective suits, consisting of cotton material, were chemically cleaned as usual in a 35 kg. naphtha plant. The centrifuged textiles were treated in 200 liters of naphtha (boiling point 140-200° C.) for 5 minutes with the addition of 24 liters of isopropanol, in which 15% of anhydrous zinc chloride and 5% of a chlorinated paraffin with a chlorine content of about 70% were dissolved. After centrifuging and drying, the treated suits were satisfactorily flameproof.

Having now particularly described the nature of the said invention and in what manner the same is to be performed, what I claim is:

1. A process for simultaneously flameproofing and cleaning textiles consisting wholly or substantially of cellulose or regenerated cellulose fibers which consists essentially of immersing said textile in a bath at a temperature of from 20° to 35° C. for from 2 to 10 minutes, said bath consisting of (1) a solution consisting of from 5% to 35% by weight of anhydrous zinc chloride in an anhy-

drous solvent selected from the group consisting of (a) lower alcohols selected from the group consisting of ethanol, propanol, isopropanol and butanol, (b) glycols selected from the group consisting of ethylene glycol, 1,2-propylene glycol and 1,3-propylene glycol, and (c) carboxylic acid esters thereof with a carboxylic acid selected from the group consisting of acetic acid and propionic acid, and (2) an organic solvent utilizable for chemical cleaning selected from the group consisting of petroleum hydrocarbons of boiling points of 80° C. to 200° C. and halogenated hydrocarbons having 1 to 4 carbon atoms, said bath having a concentration of 10 to 60 g. per liter of said anhydrous zinc chloride, removing said simultaneously fireproofed and cleaned textiles from said bath and drying said textiles.

2. A process as claimed in claim 1 in which the zinc chloride is in solution in butyl acetate.

## References Cited

## UNITED STATES PATENTS

|           |         |               |       |           |
|-----------|---------|---------------|-------|-----------|
| 1,940,668 | 12/1933 | Mohn          | ----- | 252-172   |
| 2,053,007 | 9/1936  | Parkhurst     | ----- | 252-172 X |
| 1,261,736 | 4/1918  | Ferguson      | ----- | 252-8.1   |
| 2,250,483 | 7/1941  | Hopkinson     | ----- | 117-137   |
| 2,369,200 | 2/1945  | Amerson       | ----- | 106-15    |
| 2,464,342 | 3/1949  | Pollak et al. | ----- | 117-137   |

## FOREIGN PATENTS

|         |         |               |       |        |
|---------|---------|---------------|-------|--------|
| 5,130   | 3/1905  | Great Britain | ----- | 106-15 |
| 132,813 | 11/1920 | Great Britain | ----- | 106-15 |
| 545,514 | 5/1942  | Great Britain | ----- | 106-15 |

## OTHER REFERENCES

Speel and Schwarz, Textile Chemicals and Auxiliaries, 2nd ed., Reinhold, New York, 1957, pp. 134-135.

PHILIP E. ANDERSON, Primary Examiner

D. A. JACKSON, Assistant Examiner

40 U.S. CL. X.R.

117-136; 106-15 FP; 252-8.1, 162, 172